

## UNITED STATES PATENT OFFICE

LEONARD CHESTER LORDLY, OF ELMHURST, NEW YORK

## TEXTILE PAINT

No Drawing.

Application filed October 15, 1925. Serial No. 62,648.

My invention relates to a liquid paint and medium therefor, and method of preparation of the same, which is particularly useful for incorporating color designs in the finer 5 textiles, such as silks, fine woolens, cotton and linen fabrics, etc.

In a paint for this purpose it is important that it be of a character such that it will not affect the texture or strength of the textile 10 in which it is incorporated, but will, on the contrary, leave the textile with all of its original freshness, softness, pliability and strength unimpaired. It should also be of a character such that it may be readily applied, 15 preferably by the ordinary paint brush or air brush, and capable of being localized with no substantial tendency to run or spread. Particularly it must be capable of penetrating the fabric to form a substantially 20 permanent design throughout the depth of the fabric structure, so as to form in effect an integral part thereof, appearing on both sides of textiles of the finer weave and capable of being washed or cleansed 25 without affecting or impairing the quality of the color design. The object of the invention therefore is a liquid paint which is readily applicable to textiles of the finer qualities by the ordinary paint brush and which 30 is harmless and noninjurious to the strength or texture of the fabric and moreover which can be readily applied and incorporated as a permanent part of the textile without blurring, spreading or running, the paint being 35 of a character and being prepared in a manner so as to render it readily capable of being localized and dried and the color permanently fixed or set within the design limits.

A further object of the invention is a paint 40 of the above indicated character which is capable of withstanding the severe conditions incident to the marketing and dispensing of the same and resistant for indefinite periods to impairment from changes in temperature 45 and atmospheric conditions. A further object of the invention is a paint of the above indicated character which may be economically produced and dispensed and is capable of being produced in uniform quality from 50 day to day. A further object of the inven-

tion is a medium or carrier for such a paint.

I have found that a paint suitable and entirely practicable for the above purposes can be obtained by thoroughly and intimately mixing an aniline dye of the desired color 55 with and incorporating it into gum tragacanth as a base, especially when the gum tragacanth base is treated and prepared in the manner hereinafter set forth. The gum tragacanth should be pure in quality and 60 white in color, as for example that designated in the trade as U. S. P. As a preservative to maintain the original freshness and quality of the paint for indefinite periods, it is 65 essential that some antigerm or equivalent material or ingredient also be incorporated therein, and I prefer the use of sodium benzoate for this purpose, although formaldehyde and other materials of this general 70 character might be used with more or less indifferent but unsatisfactory results, as compared to the sodium benzoate. I prefer to add to the mixture also a small proportion of acetate of aluminum which tends to fixity and fastness of the color in the texture 75 of the fabric in which the design is incorporated, although fairly satisfactory results can be obtained without the use of such ingredient. Alum or oxalic acid may be substituted for the acetate of aluminum with 80 more or less indifferent results.

The most satisfactory proportion of ingredients in the paint and the preferred method of manufacture, whereby a paint of the above indicated characteristics and these 85 proportions is obtained, are as follows—The gum tragacanth, as for example in lump form, is thoroughly washed and cleansed to remove any foreign material and substances therefrom and is then soaked in water for a 90 number of hours,—preferably overnight. The sodium benzoate and the acetate of aluminum are added and the mixture of soaked gum tragacanth, sodium benzoate and aluminum acetate is then brought to the boiling 95 point by the application of suitable heat and maintained at such boiling point for several hours, preferably two to three hours, and while at the boiling point the mixture is thoroughly agitated by stirring. To this special- 100

ly prepared gum tragacanth base, which acts as the carrier or medium for the aniline dye being used, is added the aniline dye of the proper and desired proportions and thoroughly mixed therewith as by stirring. I have found that one pound of gum tragacanth in lump form when soaked in 5 gallons of water overnight and then thus treated at the boiling temperature with 125 grams of 5 sodium benzoate and 2½ grams of aluminum acetate forms a suitable basic carrier or medium, to which water, as for example 2 gallons, may be added for diluting the specially 10 prepared gum tragacanth base before incorporating the aniline dye powder therewith. To the specially prepared base carrier or medium thus obtained may then be added aniline 15 dye powder which is thoroughly and intimately incorporated therein and mixed therewith in the proper proportions and I have 20 found that 40-60 grams of the aniline dye powder when added to 3 gallons of the specially prepared and treated base produces an entirely satisfactory paint which is practically applicable to the finer textiles and 25 usable in the above manner indicated, though of course the relative proportions of coloring matter may be varied to suit the particular requirements. Water may be added to dilute 30 the paint to the consistency desired. A paint of any shade or color may be obtained by utilizing the proper shade of aniline dye powder. The liquid paint of this character and prepared in this manner may be applied 35 to the textile by the use of the ordinary paint brush or air brush and if of the proper consistency, which may be regulated by the introduction of either water or medium (depending upon whether the paint is too thick 40 or too thin), the coating of paint, unless the coating is unduly thick, will not blur, spread or run, but will remain fixed and localized in the identical manner in which it is applied thereto by the brush. Moreover, such paint 45 is free from gluey stickiness, dries quickly after application, and does not harden or injure the texture of the textile to which it is applied.

The preferable manner of applying and 50 setting the paint on the textile is as follows: After the coating has become thoroughly dry, the painted parts of the textile are placed between two clean white cloths slightly dampened with water. The cloths should not be 55 too damp or wet for otherwise the color may be affected. The painted parts of the textile between the damp cloths are then pressed and ironed with a hot iron until dry and this operation may be repeated two or three times 60 to make sure that the color is properly set, but of course clean cloths should be utilized at each repetition. If done properly, this will set and fix the color firmly into the texture of the material and remove any surplus 65 paint or color from the surface of the textile

fabric, the ironing between the damp cloths producing a hot vapor in intimate contact with the paint and texture of the fabric. The article may be washed or dry-cleaned in the ordinary manner after this process, like any other colored fabric, and if pure mild soaps are used and proper care utilized, the color is unaffected thereby. 70

The paint of the above character and prepared in the above manner is particularly 75 suitable for textiles of silk, wool, or leather and anything of animal origin. For textiles of cotton, linen and anything of vegetable origin, the same basic medium or carrier is utilized, but instead of the acid aniline dye 80 powder a basic aniline dye of the proper proportions is to be used for thorough and intimate mixing with the specially prepared gum tragacanth base. Also for use on cotton goods there should be added to the specially 85 prepared base a small quantity of tartar emetic (chemically pure) dissolved in water or equivalent, and I prefer to use approximately 10 grams of such tartar emetic to each gallon of the specially treated and prepared 90 medium. The purpose of the tartar emetic is to neutralize the acid used in fixing and setting the color and any suitable salt effective for that purpose may be used, although I prefer the tartar emetic. Except, 95 therefore, for the use of the basic dye in the place of the acid dye and the addition of the small quantity of tartar emetic to the paint or the medium therefor for the cotton 100 textiles or fabrics and other textiles of vegetable origin, the paints for the two classes of textiles are alike.

In applying the color to cotton, linen, or goods of other vegetable origin, an acid fixative is applied to the fabric before the paint 105 is applied, and I prefer tannic acid powder dissolved in water for this purpose. This liquid coating prepares the cotton or linen material for the application of cotton colors and fixes and makes the color fast. This preparatory coating is permitted to become dry and then the paint is applied thereover to form the desired designs on the textile. The method of setting the color is then the same as described above, namely the hot ironing 115 of the same between white cloths slightly dampened until the same is dry and the operation repeated until the color is firmly fixed and set. The acid fixative may be applied after the painting operation, but I prefer the application thereof before the paint coating is applied.

The novel paint of my invention above described is transparent and is therefore particularly useful in painting designs on white textiles, but if designs are to be incorporated in colored materials, a paint of the required color to combine with that of the color of the material should be applied to obtain the resultant desired color. For example if a 120 125 130

green color design is desired on blue material, a yellow paint must be used.

While I have described my invention as being particularly applicable to incorporating color designs on the finer textiles, it is also applicable to textiles of coarser texture such as repps, sheetings and pile fabrics, and also to furs, feathers, leather, etc.

Having thus described my invention, what I claim and desire to protect by Letters Patent is:

- 10 1. A paint for forming designs on textiles consisting of a pure gum tragacanth base with sodium benzoate, acetate of aluminum, and an aniline dye thoroughly and intimately incorporated therein to form a part thereof.
- 15 2. A paint for use in incorporating color designs into the finer textiles which consists of a pure gum tragacanth base dissolved and diluted to a consistency applicable by brush and containing an aniline coloring matter and a preservative thoroughly and intimately incorporated therein to form a part thereof.
- 20 3. A medium or carrier for an aniline dye coloring matter and particularly useful in incorporating permanent color designs in the finer textiles which consists of pure gum tragacanth dissolved and treated by being brought to the boiling point and diluted to a consistency applicable by a brush and containing a preservative to preserve the freshness thereof.

In testimony whereof, I have signed my name to this specification.

L. CHESTER LORDLY.

40

45

50

55

60